

# UNITED STATES PATENT OFFICE.

HANS HOFER, OF NEW YORK, N. Y.

## METHOD OF ASSORTING SILKS.

No. 815,169.

Specification of Letters Patent.

Patented March 13, 1906.

Application filed February 3, 1905. Serial No. 244,064.

*To all whom it may concern:*

Be it known that I, HANS HOFER, of the Republic of Switzerland, residing in New York, county and State of New York, have 5 invented certain new and useful Improvements in Methods of Assorting Silks; and I do hereby declare the following to be a full, clear, and exact description of the invention, such as will enable others skilled in the art to which 10 it appertains to make and use the same.

This invention has for its object to make certain raw silks, such as China Tsatlee filatures or China native filatures, available generally for industrial purposes—that is to say, 15 for the manufacture of broad silk goods, narrow-ware goods, &c.—as well as for embroidery and sewing purposes. The great bulk of the China raw silks being prepared by the natives according to crude and primitive 20 methods cannot be used for weaving purposes, or, indeed, any other purposes where regularity in size is essential not only with respect to the ultimate quality of the product, but with respect to the operation of the 25 machinery employed in developing it. Such silks are almost exclusively used only for sewing and embroidery, the silks employed in weaving and other arts where uniformity is essential being those which are produced and 30 prepared in and according to the modern methods of Europe and Japan. The crude native method of preparing China silks results in such diversities of gage or thickness of filaments that in one bale of silk the size 35 often varies from fifteen to fifty and more deniers in single-filament silk, and such irregularity becomes all the more apparent if the two extremes of size happen to join, as is often the case.

40 My invention is a method of assorting silks of materially-diversified sizes which consists in weighing the silk in the filament and in comparatively short lengths at a time, then dividing it into separate lots each comprising

lengths of filament having approximately the 45 same weight, and then joining those lengths of filaments having approximately the same weight together to make a single thread thereof. The result is that in each lot the different filaments will be found to be approximately for all practical purposes of the same 50 number of sizes, (deniers,) which are thus merchantable as of a uniform size for use generally in the manufacture of silk goods of whatever description. When thus assorted, the 55 filaments found to be of the same size may be combined by throwing to form a single thread and otherwise manipulated to put them in condition for the particular use to which the silk is to be put.

My invention is of peculiar value because it makes now available silks which are recognized as being naturally the most lustrous and in certain other respects the best silks known.

Having thus fully described my invention, what I claim as new, and desire to secure by Letters Patent, is—

The method of assorting silks of different sizes or thicknesses into lots comprising filaments all of substantially the same size or thickness which consists in weighing the silk in the filament, and in comparatively short lengths at a time, then separating those lengths of filament having approximately the 70 same weight from the remainder, and then joining those lengths of filaments having approximately the same weight together to make a single thread thereof, substantially as 75 described.

In testimony that I claim the foregoing I have hereunto set my hand this 1st day of February, 1905.

HANS HOFER.

Witnesses:

JOHN W. STEWARD,  
WM. D. BELL.